

(No Model.)

J. E. & H. E. HARTLEY.  
ATTACHABLE LETTER FOR SIGNS.

No. 488,655.

Patented Dec. 27, 1892.

FIG 1



A.

FIG 2



Witnesses.

Ernest W. Jones.

Wilfrid C. Bragge.

Inventors.

John Edward Hartley.

Herbert Edward Hartley

Rev. Charles J. Powell

Attorney

# UNITED STATES PATENT OFFICE.

JOHN EBORALL HARTLEY AND HERBERT EDWARD HARTLEY, OF  
BIRMINGHAM, ENGLAND.

## ATTACHABLE LETTER FOR SIGNS.

SPECIFICATION forming part of Letters Patent No. 488,655, dated December 27, 1892.

Application filed June 7, 1892. Serial No. 435,906. (No model.)

*To all whom it may concern:*

Be it known that we, JOHN EBORALL HARTLEY and HERBERT EDWARD HARTLEY, subjects of the Queen of Great Britain, both residing at 13 Saint Paul's Square, Birmingham, England, have invented certain new and useful Improvements in Attachable Letters for Signs, (for which we have applied for Letters Patent in England, No. 191, dated January 5, 1892;) and we do hereby declare that the following is a full, clear, and exact description of the invention, which will enable others skilled in the art to which it appertains to make and use the same.

15 This invention relates to the manufacture of letters, including of course numerals or other similar figures, used for signs, and its object is to combine with a cast body of lead and antimony such letters the following processes, first, of an electro-deposition of copper, to be followed by an electro deposition of gold or of silver, which is then coated with any of the well known coatings of celluloid, and further in combining with the last 25 named process, a further coating of seed-lac varnish.

We carry our invention into effect in the manner illustrated in the accompanying drawings in which:—

30 Figure 1, is a view in elevation of a letter to which our improved process is applied. Fig. 2, is an enlarged cross sectional plan view on line 1, 1, Fig. 1.

We provide what are known as chill molds, 35 which are preferably made of metal, but may be made of plaster of paris, the object being to obtain a perfectly smooth surface. We then melt an alloy composed of five parts by weight of lead and one part by weight of antimony, from which the letter A is cast. The difficulty experienced in obtaining an alloy for casting these letters has been to get cheap alloy that will flow freely when fused, and afford a smooth surface free of air holes, 40 when cold. The alloy herein stated we find to answer these purposes satisfactorily. These

letters are now pickled and cleaned by the present well known methods ready for the electro plating bath. They are then treated with an electro deposition of copper B as a base, and further with a subsequent electro deposition of gold or of silver C. These depositions are now protected by a film D of celluloid applied in any of the ordinary methods. Similar surfaces when thus only protected by this film D of celluloid, as is the present custom, are open to the objection that the film is liable to chip, particularly at the edges, and especially should the articles so coated be subject to frictional wear. In order to avoid this however, we add a further coating of colorless, or as near colorless as may be, cold drying seed-lac varnish E. This we find to effectually prevent such chipping or peeling, and very much increasing the duration of the brilliancy of the letters.

The forms and sectional shapes of the letters, may of course be varied and also by letters we include numerals or such similar figures analogous to letters, used for sign board purposes.

We are aware of various alloy compositions for casting purposes in which antimony and lead have been used. Also we are aware that a film of celluloid has been already applied to preserve metallic surfaces from atmospheric, gaseous or acidiferous action, also that the process of electro deposition in itself is old, and therefore we do not claim those processes or the composition broadly; but

What we do claim as new and desire to secure by Letters Patent is:—

In sign letters, numerals &c, the combination with the cast metal body, of the coating of copper, and the coating of precious metal and the films of celluloid and seed-lac varnish, substantially as described.

JOHN EBORALL HARTLEY.  
HERBERT EDWARD HARTLEY.

Witnesses:

CHARLES T. POWELL,  
ERNEST W. JONES.